

Nov. 3, 1925.

1,560,106

W. E. SHEENE

## ASPHALT VAULT

Filed May 7, 1924



WITNESSES  
Porter St. Lauts,  
E. Wehineyer

William E. Sheene Inventor

By Edwin F. Daniels

### mentor

Attorney

Patented Nov. 3, 1925.

1,560,106

# UNITED STATES PATENT OFFICE.

WILLIAM E. SHEENE, OF BALTIMORE, MARYLAND, ASSIGNOR TO THE ASPHALT GRAVE VAULT COMPANY, A CORPORATION OF MARYLAND.

## ASPHALT VAULT.

Application filed May 7, 1924. Serial No. 711,518.

To all whom it may concern:

Be it known that I, WILLIAM E. SHEENE, a citizen of the United States of America, residing in the city of Baltimore, State of Maryland, have invented certain new and useful Improvements in Asphalt Vaults, of which the following is a specification.

Numerous attempts have been made to produce a permanent moisture-proof burial vault or container to receive and enclose a coffin or casket to be buried in the earth, the object being not only to exclude moisture but to permanently protect and preserve the coffin and the body.

To this end the structure must not only be water-proof but non-corrosive and sufficiently rigid to permanently resist the pressure of the earth. Such containers have been made from metal, Portland cement, concrete with or without reinforcement, and from metal lined or filled with asphalt, the asphalt being between two metallic casings or walls.

The Portland cement concrete is not effective because while it is reasonably permanent, it is porous and not water-proof, and the entrance of moisture results in decay which cannot be long deferred. The metallic vaults are not permanent, none of the available metals being sufficiently non-corrosive. The vaults which have been described as made of asphalt between metal walls or in some instances enclosed between walls of wood, are subject to substantially the same objections as the metallic vaults in that the outer wall disappears in a comparatively short time, and the asphalt which in accordance with the specifications is necessarily soft and relatively fluid, owing to its fluidity soon leaves the inner container or casing exposed to decay or corrosion, which takes place as certainly as with metal or wooden vaults, though the decay may be deferred for several years.

The present invention relates to an asphalt vault or more particularly to an asphalt or bituminous mastic for the manufacture of a vault meeting all the requirements of the conditions presented, i. e., a vault for enclosing a casket and body to be buried in the earth and having sufficient rigidity to resist permanently the pressure of the earth, and being absolutely moisture-proof. In my co-pending application Ser. No. 711,519, I have described and claimed

a reinforcing frame for an asphalt vault, the same being coated with asphalt to complete the structure. In the present application I have described and claimed an asphalt vault, the claims being specific to such a structure composed of asphalt which is sufficiently rigid to resist the earth pressure when suitably reinforced, claiming the constituents, properties and features of the vault as dependent upon the asphaltic material.

The mastic which is the subject of the invention is cast upon a metal frame or reinforce which shapes and supports the structure, the important features of the mastic are that in addition to being capable of being melted, poured and molded to advantage, it is, when set, sufficiently hard to adhere to the frame and to resist and support the pressure of the earth upon the frame, spanning the meshes of the reinforce and being practically non-fluid at the temperatures and pressures of the earth, the resistance thus presented by this material being positive and permanent so that the mastic affords a permanent covering for the reinforce and a permanent protection to the casket and body, and the mastic is at the same time absolutely and permanently moisture-proof, so that the most hydroscopic and sensitive substances may be placed on the bottom of the container or vault, and the vault can be submerged for a long period without evidence of the hydroscopic substances thus exposed having been in any way attacked by moisture.

In the preferred form the mastic consists of a high melting point asphalt mixed with limestone dust, fuller's earth or infusorial earth and sand or grit. In some instances slate dust has been used instead of limestone dust. In preparing the composition I preferably use a blown asphalt which may to best advantage be made of petroleum or petroleum residue heated and blown until the volatile portions are practically eliminated or oxidized, and until the resulting material has a melting point approaching 285° Fahrenheit when it will also have the desired property of rigidity when mixed with the appropriate ingredients and permitted to set or harden and subjected to the earth temperatures and pressures under burial conditions. A California or Mexican petroleum or residue thus treated is found

satisfactory. The preferred proportions are 16% bitumen or asphalt as above, 34% limestone dust, fuller's earth or infusorial earth, and 50% of sand or other suitable 5 grit. The materials and proportions may be varied to a considerable degree, and a flux which does not unduly interfere with the hardness of the material when set may be used.

10 The materials stated above are mixed together and cooked, or preferably separately heated, and then mixed and further heated until they form a paste or mortar capable of being poured and molded. Treatment at 15 a temperature of 450° Fahrenheit has been found advantageous.

A suitable reinforce having the shape of the vault or rather two separate reinforcing members, one having the shape of the vault 20 and the other having the shape of a cover, are placed in molds, and the material is poured, hardening in the desired form.

In the accompanying drawing I have 25 illustrated the essentials of a vault embodying my invention in the preferred form.

In the drawing—

Figure 1 is a longitudinal vertical section showing the vault enclosed and buried in the ground, the coffin being indicated 30 therein in dotted lines.

Figure 2 is a perspective view of the cover reinforce; and

Figure 3 is a section on the line 3, 3 of Figure 2.

35 Referring to the drawings by numerals, each of which is used to indicate the same or similar parts in the different figures, the illustration includes a vault 1 of asphalt mastic adapted to enclose a single coffin or 40 casket 2, and a cover 3, also of asphalt mastic, the vault and cover being reinforced by means of metal frames 4 and 5, respectively, embedded in and protected by the mastic. The contact between the vault and cover is 45 closed and sealed by suitable sealing means 6 of softer bitumen or asphalt adhering to adjacent asphaltic surfaces of the vault and cover, making the structure, when closed permanently, air and moisture-proof 50 at all points, which is believed to be a result not previously attained in burial containers of this general type.

More particularly the vault reinforce 55 consists of longitudinal angle irons 8 extending along the top edges of each side, transverse angle irons 9 extending across the bottom and up each side, and end angles 10 extending vertically across the ends and turned under the bottom, so that they cross the 60 transverse angles 9, the depending flanges of the end angles being cut away at 11 to pass the transverse angles. The vertical angles 10 and the transverse angles 9 are connected by reinforcing rods or wires 14 65 which are in turn connected by upright

wires or rods 15, the intersections in all instances being preferably spot-welded or otherwise fastened.

In the form shown the wires are omitted at the bottom and there is a plate 16 which may be turned up at the edges at 17, and which reinforces the entire bottom, the plate being preferably separate from the other reinforce.

The cover reinforce consists of angles 18 75 extending longitudinally at the sides and transversely at 19 at the ends, the members 18 and 19 being preferably formed in a single piece, the transverse angles 20 and longitudinal and transverse wires or rods 21 80 and 22.

The cover and vault are formed by placing these frame members in suitable molds, pouring and removing the mold members.

Important features of the invention are 85 that the mastic described is not only absolutely moisture-proof but is sufficiently hard when set to resist the pressure of the earth on the vault between the rigid reinforcing members, being absolutely non-fluid 90 at earth temperatures and therefore retaining its form and protecting the frame and reinforce permanently without yielding in any way.

The term burial conditions, as used herein, refers to conditions to which the casket and vault enclosing the casket are subjected when placed in the ground at the average depth of burial and covered with earth, the grave being filled to the depth of the top 95 surface of the soil, in accordance with the usual practice.

I have thus described specifically and in detail an ashpalt mastic burial vault embodying the features of my invention in the 100 preferred form in order that the nature and operation of the same may be clearly understood; however, the specific terms herein are used descriptively and not in a limiting sense, the scope of the invention being 105 defined in the claims.

What I claim and desire to secure by Letters Patent is:

1. A moisture-proof burial vault to be buried in the ground to enclose and preserve 115 a casket and the body therein, the vault structure having walls composed of bituminous mastic consisting of infusorial earth, grit and bitumen and a frame embedded in the mastic and protected thereby, reinforcing 120 the walls and forming a permanent structure at the temperatures and pressures to which it is subject under the conditions of burial.

2. A moisture-proof burial vault to be 125 buried in the ground to enclose and preserve a casket and the body therein, the vault having walls composed of bituminous mastic consisting of infusorial earth, grit and bitumen, the bitumen having a melting point 130

of approximately 285° Fahrenheit and the mastic being hard and non-fluid at earth temperatures and pressures, and a frame embedded in the mastic and protected thereby, 5 reinforcing the walls.

3. A moisture-proof burial vault to be buried in the ground to enclose and preserve a casket and the body therein, the vault structure having walls composed of 10 a mastic consisting of bitumen having a melting point of approximately 285° Fahrenheit and being more than one-half composed of filler, and a frame embedded in the mastic and protected thereby, reinforcing 15 the walls, and forming a permanent structure at the temperatures and pressures to which it is subject under the conditions of burial.

4. A moisture-proof burial vault adapted to be buried in the ground to enclose and protect a burial casket and the contents, the vault having a frame and being otherwise composed of bituminous mastic, the frame being embedded in and protected by the 20 bituminous material which is permanent, non-fluid and substantially rigid at the earth temperatures and pressures to which it is subjected under burial conditions.

5. A burial vault adapted to enclose a 30 coffin or casket and to be buried in the ground, the same comprising a metallic reinforcing frame and a hard asphalt mastic wholly non-fluid at earth temperatures consisting of bitumen having a melting point 35 of approximately 285° Fahrenheit and a

filler, the mastic containing approximately 16% bitumen, 50% gritty material and 34% of other filler.

6. A burial vault adapted to enclose a coffin or casket and to be buried in the ground, the same comprising a metallic reinforcing frame covered by and enclosed within a hard asphalt mastic, non-fluid at earth temperatures, consisting of bitumen having a high melting point and a filler, 40 the mastic containing approximately 16% bitumen, 34% fuller's earth and 50% grit.

7. A container for a casket to be buried in the ground, the same consisting of a vault and a cover, both being molded of hard 50 asphaltic material and a seal of softer asphaltic material connecting the vault and cover, and adhering to adjacent asphaltic surfaces of the vault and cover.

8. A moisture-proof burial vault adapted to be buried in the ground, to enclose a burial casket and the contents, the vault having a frame and being otherwise composed of bituminous mastic, the same consisting of approximately three-fourths filler and one-fourth bitumen, the frame being embedded in and protected by the bituminous material which is permanent, non-fluid and substantially rigid at earth temperatures and the pressures to which it is subjected under ordinary burial conditions. 60 65

Signed by me at Baltimore, Maryland, this 15th day of April, 1924.

WILLIAM E. SHEENE.